

April 28, 1925.

1,535,893

M. BELCHER

PUMP VALVE

Filed May 27, 1924



Fig. 1.



Fig. 2.



Fig. 3.

M. Belcher Inventor

By Jesse R. Stone  
his Attorney

## UNITED STATES PATENT OFFICE.

MARK BELCHER, OF DAISETTA, TEXAS.

## PUMP VALVE.

Application filed May 27, 1924. Serial No. 716,104.

*To all whom it may concern:*

Be it known that I, MARK BELCHER, a citizen of the United States, residing at Daisetta, Texas, have invented a certain new and useful Improvement in Pump Valves, of which the following is a specification.

My invention relates to valves such as are employed in pumps designed for handling mud, water, and liquids carrying sand or sediment tending to wear the valves.

In mud pumps such as are employed in well drilling operation, the pump must handle large quantities of muddy fluid employed in flushing out the material disintegrated by the drill. The mud ordinarily has, in suspension therein, large quantities of sand and abrasive material tending to wear the valves. The valves are worn so quickly that they must be repacked or renewed so frequently as to necessitate employing extra pumps to be used when others are being repaired. A large amount of valuable time and material are thus lost in maintaining the pumps in operating condition.

It is an object of my invention to provide a valve which will resist wear for long periods of time under the conditions of wear to which mud pumps are subjected.

It is another object to provide a pump valve which will not be detrimentally affected by the action of salt water or acids occasionally encountered in drilling oil or sulphur wells.

It is also desired that it be capable of maintaining a tight fit in its seat without the necessity of packing.

In carrying out my invention I employ certain species of hard, tough wood which must be specially treated; and the process of treatment to which the wood is subject comprises an important part of my invention.

Referring to the drawings herewith, Fig. 1 is a perspective view of a wooden disc comprising the body of my valve member. Fig. 2 is a broken view partly in section through a pump of the character referred to, in which my valve is employed. Fig. 3 is a central vertical section through a slightly modified valve. Like numerals of reference are employed to designate like parts in all the views.

In the ordinary type of so-called gumbo buster mud pump, the valve 1 is disc shaped and seats upon a ring 2 fitting within a seat 3 in the pump 4. The valve 1 is slidable

on a rod 5 and is held resiliently in its seat by a spring 6 bearing at its upper end against the discharge valve cover 7 which also retains the upper end of the valve rod 5.

The ordinary valve employed in this type of pump is metal packed with some compressible composition such as rubber or rubberized fabric. I have found that a wooden disk, properly selected and treated will be much more lasting and satisfactory.

I select a tree of hard wood such as sweet gum, hickory, or pecan. It is well in young trees to select only the lower end adjacent the ground. This portion is thoroughly seasoned which may be done by peeling the bark from the lower end of the tree and allowing the tree to stand uncut until it is thoroughly dry. I may, however, season the piece by placing it in a bath of salt water and keeping it submerged therein for several months. I usually treat the wood in brine for about six months.

I obtain good results by selecting trees which can be turned down to the proper diameter with very little labor, and after the wood has been thoroughly treated it is turned in a lathe to about the proper diameter of the valve which is to be constructed. About one-eighth of an inch is allowed for shrinkage. The block is then cut up into discs of about one and one-fourth inches in thickness, and the outer face of each disc, is slightly curved so that it is slightly smaller in diameter at each end to allow for a proper seating of the valve without obstruction.

The discs thus cut into proper shape are then put in a container having linseed oil therein and thoroughly soaked for about twenty-four hours. The discs are then removed and placed in a bath composed of about one-half linseed oil and one-fourth each of lead and graphite. This mixture is thoroughly heated and the discs are submitted to a boiling temperature while in this charge for about fifteen minutes and then are allowed to cool.

The discs are thus in shape to use except for a hardening treatment for which they are further subjected. I find that by submitting the outer surface of the disc to a burning temperature so that the outer surface is slightly charred by the heat, the wood is not only better preserved and hardened,

but will have a velvety texture which makes it form a better seat in its pumping operations. The charring of the surface is not sufficient to remove any material portion of the wood, and may best be done by placing the disc upon a red hot metallic surface for a very short period. The disc is then smoothed slightly with sand paper or other similar treatment, and is ready for use. A 10 central opening 8 is bored through the center thereof to receive the valve stem.

If the disc is to be used in ordinary mud pumps the valve is sufficiently strong to withstand any rough usage to which it may 15 be put for long periods of time. If the valve is to be used with high pressure pumps in which high pressures are employed, it is desirable in some instances to reinforce the disc somewhat to prevent cracking or 20 splitting under the strain of the excessive pressure. In such cases I employ an open cap or ring 9, such as is shown in Fig. 3, fitting over the upper end of the disc and setting down around the periphery thereof 25 for a short distance sufficient to prevent splitting or cracking of the disc. I may set the ring 9 into the side of the disc so that it will come flush with the outer face thereof, as shown in the drawing. The lower 30 face of the disc is thus formed of the hard wood treated as above set forth. A contacting surface between the disc and the ring 2 forming the seat thereof is therefore made with the charred lower face of 35 the disc and the close fitting between the parts will be accomplished, which will not be easily worn by the sand or mud, and will endure for a much longer period than will the ordinary packing now employed. 40 It will also be obvious that a disc of this kind is not affected materially by acids or salt water, and for this reason will function more effectively than the usual metal or composition disc.

45 In the formation of a valve disc such as described, it is contemplated that different hard woods will be employed and that after seasoning in the manner set forth, such wood will be submitted to the process 50 of treatment described. I do not wish, however, to be confined to the exact method of treatment further than is set forth in the claims appended hereto; it being obvious that various changes may be made 55 in the process of formation of the valve disc without departing from the spirit of the invention.

Having thus described my invention, what

I claim as new and desire to protect by Letters Patent is:

1. A process of treating pump valves of hard wood comprising, thoroughly seasoning said valves, submitting them to the action of a preservative under heat, charring the outer face thereof and smoothing the 65 charred surface.

2. A process of treating wooden valve discs of hard wood comprising, thoroughly seasoning the wood, soaking the discs in linseed oil for approximately twenty-four 70 hours, then boiling the same in a mixture composed of approximately one-half linseed oil, one-fourth white lead, and one-fourth graphite, and then charring the outer surface.

3. A process of treating wooden valve discs comprising, soaking the wood in a bath of salt water for a period of several months, soaking the discs in a bath of linseed oil, then boiling the same in linseed 80 oil, white lead and graphite, and then charring the lower face for the purpose described.

4. A process of forming a valve disc comprising, seasoning hard wood for a sufficient period, sawing the wood into discs of the proper size, soaking the same in linseed oil, then boiling said discs in linseed oil, white lead and graphite, and submitting the outer surface of the disc to the 85 action of dry heat.

5. A process of forming valve discs for mud pumps comprising thoroughly seasoning the wood, soaking the discs for several hours in linseed oil, boiling the discs in 90 equal parts of graphite and white lead mixed with oil, charring the outer surface of the discs and smoothing the lower surface.

6. A process of forming valve discs for 100 mud pumps comprising, cutting hard wood into discs of the desired form, soaking said discs in linseed oil, then boiling said discs in a mixture of linseed oil, graphite and lead, charring the outer surface, and smoothing the lower face.

7. A process of forming valve discs for mud pumps comprising, cutting hard wood into discs of the desired form, thoroughly impregnating said discs with oil, charring 110 the outer surface thereof, and smoothing the working faces of said discs.

In testimony whereof I hereunto affix my signature this 22nd day of May, A. D. 1924.

MARK BELCHER.